

(No Model.)

J. A. POTTER.  
MODE OF SHAPING CAST STEEL.

No. 434,294.

Patented Aug. 12, 1890.



WITNESSES

*H. L. Gill*  
*N. B. Conover*

INVENTOR

*John A. Potter*  
*by his attorney*  
*T. Dakewell & Sons*

# UNITED STATES PATENT OFFICE.

JOHN A. POTTER, OF HOMESTEAD, PENNSYLVANIA.

## MODE OF SHAPING CAST-STEEL.

SPECIFICATION forming part of Letters Patent No. 434,294, dated August 12, 1890.

Application filed December 5, 1889. Serial No. 332,676. (No model.)

*To all whom it may concern:*

Be it known that I, JOHN A. POTTER, of Homestead, in the county of Allegheny and State of Pennsylvania, have invented a new and useful Improvement in Shaping Cast-Steel, of which the following is a full, clear, and exact description.

My invention relates to an improvement in the art of shaping cast-steel for the production of articles of dense and homogeneous structure free from blow-holes and of great strength, and is illustrated in the accompanying drawing, which shows a side elevation, partly in section, of apparatus which I have devised for the practice of the invention. This drawing shows a mold of proper shape to produce a steel cannon, for the manufacture of which my invention is especially well adapted; but it will be understood that the invention, as hereinafter defined in the claims, has other uses, and may be applied to the shaping of other articles, such as shafting, &c.

In the drawing, 2 represents a mold, which is preferably made of a single cast piece of metal having a mold-cavity 3, whose internal shape conforms to the article to be produced, and having at the end of the mold-cavity, and directly communicating therewith, a cavity 8, in which the end of a ram 4 fits and works. This ram 4 is set on or secured to a plunger 1, which works within a hydraulic cylinder 5, the ram being removably set on the plunger for the purpose of enabling the cylinder and plunger to be used with molds of different sizes, as hereinafter explained. The cylinder 5 is in line with the mold-cavity and is preferably secured thereto by strong tie-bolts 6, 7 being a guide-plate or ring interposed between the mold and cylinder and fitting neatly around the ram. Both the ram and the mold may be suitably water-cooled by internal water-circulating passages or pipes.

15 is the supply-pipe which admits water to the cylinder 5 at the outer end of the plunger.

45 9 is a ladle supported by a suitable crane 10, and adapted to supply molten steel to the mold. The mold-cavity is open at the end opposite to the plunger and in form the cavity tapers in diameter toward the open end.

50 The operation is as follows: The parts being in the position shown in the drawing, the ladle 9 is carried by the crane into position

above the open end of the mold, and the steel is poured into the cavity in quantity sufficient to form the article desired to be made. A 55 plate or cover 11 (shown by dotted lines in the drawing) is then placed over the mouth of the mold, and secured thereon by a bar 12 passing over the cover through lugs 13 on the mold and by a wedge 14 between the bar and 60 cover. The ram 4 is then raised within the mold-cavity, so as to force the metal up into the narrower cavity 3, and to compress it against the cover, the effect of which compression is to densify the metal, to render its 65 heat uniform throughout, and to expel therefrom the gases, which escape from the mold through perforations or air-passages which may be formed in the cover. The metal is thus maintained in a state of compression 70 against the cover until by radiation of its heat it loses its fluidity and solidifies. By thus suffering the metal to cool under compression it is caused to shrink uniformly, a uniform 75 temperature throughout the whole mass is maintained, and segregation into pockets of the non-metallic constituents—such as carbon and phosphorus—is effectually prevented. When the metal has properly solidified, the fastening of the mold-cover is removed and 80 further pressure is applied by the ram to the metal, the effect of which is to discharge the metal from the cavity 8, forcing it up in the contracted cavity 3 and causing the surplus to lift the cover and to protrude from the open 85 end of the mold. As said cavity, by reason of its contracted shape, opposes resistance to the advance of the metal, it exerts thereon a reducing and compressing action, which has the effect of still more densifying its composition, 90 increasing its strength, and rendering it homogeneous. The advance of the ram is continued until it reaches the end of the cavity 8, and when the shaping is thus completed the plunger and ram are retracted, and by removing the mold from the plate 7 and allowing the metal to cool sufficiently to shrink loose from the mold it may be removed or ejected in any suitable way.

By reason of the construction of the parts 100 above described and shown, it follows that the same cylinder 5 and plunger 1 may be employed in connection with molds of various sizes and shape, all that is necessary to adapt

them to a new mold being to replace the ram with one of proper size to fit the mold-cavity 8, and the plate 7 with one having a hole of proper diameter to fit neatly around the ram, 5 so as to prevent possibility of the escape of metal when the mold is in use.

Various modifications of the apparatus may be made without departing from the principles of my invention as herein claimed. For 10 example, the construction and arrangement of the hydraulic mechanism may be varied, and the mold, instead of being made in a single piece, may be formed of several pieces, which may be held together by a hydraulic 15 ram or otherwise.

Other modifications will suggest themselves to the skilled mechanic.

The advantages of my invention will be appreciated by those skilled in the art. Articles produced as above described are of great 20 strength and superior quality, and the cost of the construction and operation of the apparatus is small as compared with the saving and benefits attained by its use.

25 The essential features of my invention consist, first, in producing a forging by forcing steel by pressure from a larger cavity of a mold into a smaller cavity, thus reducing and densifying the same; second, in subjecting 30 molten steel to compression in a mold, permitting it to solidify therein, and then by pressure causing it to pass in through a mold-cavity of contracted diameter, the contraction of such cavity preferably being gradual, and, 35 third, in the apparatus shown in the drawing and the several integral parts thereof.

I claim—

1. In the art of shaping cast-steel, the im-

provement which consists in charging molten steel into a cavity of contracting cross-section, permitting it to solidify therein, and then forcing it through such cavity, whereby the metal is laterally reduced and compacted, substantially as and for the purposes described. 40

2. In the art of shaping cast-steel, the improvement which consists in charging molten steel into a mold-cavity of contracting cross-section, compressing it therein and permitting it to solidify under such compression, and then forcing the solidified and compressed 50 metal through such cavity, whereby the metal is laterally reduced and forged, substantially as and for the purposes described.

3. The combination of the mold having a cavity 8 for receiving molten steel, a contracted cavity having an open end, and a hydraulic cylinder and ram, substantially as 55 and for the purposes described.

4. The combination of the mold having a cavity 8 for receiving molten steel, a contracted cavity, and a hydraulic cylinder and ram, and a plate 7, which fits around the ram, substantially as and for the purposes described. 60

5. The combination of the mold having a cavity 8 for receiving molten steel, a contracted cavity having an open end, a hydraulic cylinder and ram, and a removable cover, substantially as and for the purposes 65 described. 70

In testimony whereof I have hereunto set my hand this 2d day of November, A. D. 1889.

JOHN A. POTTER.

Witnesses:

W. B. CORWIN,  
JNO. K. SMITH.